



| (56)                  | References Cited           |                                                                                                                                              |            |                  |          |  |  |
|-----------------------|----------------------------|----------------------------------------------------------------------------------------------------------------------------------------------|------------|------------------|----------|--|--|
| U.S. PATENT DOCUMENTS |                            |                                                                                                                                              |            |                  |          |  |  |
| 3,956,283 A           | 5/1976 Fleck               | 2009/0297738 A1*                                                                                                                             | 12/2009    | Song et al. .... | 428/32.3 |  |  |
| 4,371,582 A           | 2/1983 Sugiyama et al.     | 2009/0320708 A1                                                                                                                              | 12/2009    | Jackson et al.   |          |  |  |
| 4,440,827 A           | 4/1984 Miyamoto et al.     | 2010/0028659 A1                                                                                                                              | 2/2010     | Shimono et al.   |          |  |  |
| 4,721,655 A           | 1/1988 Trzasko             | 2010/0129553 A1                                                                                                                              | 5/2010     | Jackson et al.   |          |  |  |
| 4,806,207 A           | 2/1989 Monzon et al.       | 2011/0151148 A1                                                                                                                              | 6/2011     | Koenig et al.    |          |  |  |
| 5,000,797 A           | 3/1991 Honkura et al.      | 2011/0151149 A1                                                                                                                              | 6/2011     | Koenig           |          |  |  |
| 5,043,017 A           | 8/1991 Passaretti          | 2011/0240241 A1                                                                                                                              | 10/2011    | Koenig et al.    |          |  |  |
| 5,164,006 A           | 11/1992 Chapnerkar et al.  | 2011/0240242 A1                                                                                                                              | 10/2011    | Koenig et al.    |          |  |  |
| 5,254,403 A           | 10/1993 Malhotra           | 2011/0274856 A1                                                                                                                              | 11/2011    | Koenig et al.    |          |  |  |
| 5,281,467 A           | 1/1994 Shimada et al.      | 2012/0019587 A1                                                                                                                              | 1/2012     | Koenig           |          |  |  |
| 5,397,619 A           | 3/1995 Kuroyama et al.     | 2012/0121872 A1                                                                                                                              | 5/2012     | Koenig           |          |  |  |
| 5,429,860 A           | 7/1995 Held et al.         | FOREIGN PATENT DOCUMENTS                                                                                                                     |            |                  |          |  |  |
| 5,531,821 A           | 7/1996 Wu                  | EP                                                                                                                                           | 1036666    | 9/2000           |          |  |  |
| 5,593,488 A           | 1/1997 Wu                  | EP                                                                                                                                           | 1079356    | 2/2001           |          |  |  |
| 5,593,489 A           | 1/1997 Wu                  | EP                                                                                                                                           | 1122085    | 8/2001           |          |  |  |
| 5,599,388 A           | 2/1997 Wu                  | EP                                                                                                                                           | 1355004    | 10/2003          |          |  |  |
| 5,643,631 A           | 7/1997 Donigian et al.     | EP                                                                                                                                           | 1566281    | 8/2005           |          |  |  |
| 5,686,602 A           | 11/1997 Farooq et al.      | EP                                                                                                                                           | 1571149    | 9/2005           |          |  |  |
| 5,711,799 A           | 1/1998 Snowden et al.      | EP                                                                                                                                           | 1712677    | 10/2006          |          |  |  |
| 5,783,038 A           | 7/1998 Donigian et al.     | EP                                                                                                                                           | 1743976    | 1/2007           |          |  |  |
| 5,851,651 A           | 12/1998 Chao               | EP                                                                                                                                           | 1775141    | 4/2007           |          |  |  |
| 5,858,555 A           | 1/1999 Kuroyama et al.     | EP                                                                                                                                           | 1947240    | 7/2008           |          |  |  |
| 5,965,244 A           | 10/1999 Tang et al.        | JP                                                                                                                                           | 2002274012 | 9/2002           |          |  |  |
| 6,083,317 A           | 7/2000 Snowden et al.      | JP                                                                                                                                           | 2004255593 | 6/2004           |          |  |  |
| 6,139,961 A           | 10/2000 Blankenship et al. | JP                                                                                                                                           | 2006168017 | 6/2006           |          |  |  |
| 6,150,289 A           | 11/2000 Chen et al.        | WO                                                                                                                                           | 9609345    | 3/1996           |          |  |  |
| 6,162,328 A           | 12/2000 Cennisio et al.    | WO                                                                                                                                           | 9906219    | 2/1999           |          |  |  |
| 6,207,258 B1          | 3/2001 Varnell             | WO                                                                                                                                           | 9916973    | 4/1999           |          |  |  |
| 6,623,819 B2          | 9/2003 Missell et al.      | WO                                                                                                                                           | 03044275   | 5/2003           |          |  |  |
| 6,626,531 B2          | 9/2003 Fujii et al.        | WO                                                                                                                                           | 2005115763 | 12/2005          |          |  |  |
| 6,656,545 B1          | 12/2003 Schliesman et al.  | WO                                                                                                                                           | 2006049545 | 5/2006           |          |  |  |
| 6,764,726 B1          | 7/2004 Yang et al.         | WO                                                                                                                                           | 2006110751 | 10/2006          |          |  |  |
| 6,777,041 B2          | 8/2004 Yau et al.          | WO                                                                                                                                           | 2007053681 | 5/2007           |          |  |  |
| 6,808,767 B2          | 10/2004 Schliesman         | WO                                                                                                                                           | 2007141271 | 12/2007          |          |  |  |
| 6,979,481 B2          | 12/2005 Gaynor et al.      | WO                                                                                                                                           | 2008055858 | 5/2008           |          |  |  |
| 6,984,423 B2*         | 1/2006 Iida et al. ....    | WO                                                                                                                                           | 2008124731 | 10/2008          |          |  |  |
| 7,255,910 B1          | 8/2007 Seckel              | WO                                                                                                                                           | 2009110910 | 9/2009           |          |  |  |
| 7,297,382 B2          | 11/2007 Van Aert et al.    | WO                                                                                                                                           | 2009124075 | 10/2009          |          |  |  |
| 7,303,794 B2          | 12/2007 Superka et al.     | WO                                                                                                                                           | 2009146416 | 12/2009          |          |  |  |
| 7,521,101 B2          | 4/2009 Naisby et al.       | OTHER PUBLICATIONS                                                                                                                           |            |                  |          |  |  |
| 7,559,643 B2          | 7/2009 Chen et al.         | Quantitative Determination of Alkyl Ketene dimer AKD retention in Paper made on a Pilot Paper Machine, p. 253-260.                           |            |                  |          |  |  |
| 7,582,188 B2          | 9/2009 Stoffel et al.      | Automataic Color recognition System for Stockigt Sizing Test II, Journal of Korea TAPPI, 371-73-81, 2005.                                    |            |                  |          |  |  |
| 7,618,692 B2          | 11/2009 Nakano et al.      | C. E. Farley; R. B. Wasser. The Sizing of Paper. TAPPI Press, 1989, 51-62.                                                                   |            |                  |          |  |  |
| 7,638,176 B2          | 12/2009 Kasperchik et al.  | Paper and board—Determination of sizing—Stoeckigt method, JIS P 8122- 2004, rev. Mar. 20, 2004, published by Japanese Standards Association. |            |                  |          |  |  |
| 7,651,216 B2          | 1/2010 Chen et al.         | Chemistry and Application of Rosin Size, E. Strazzins, pp. 1-31.                                                                             |            |                  |          |  |  |
| 7,651,747 B2          | 1/2010 Chen et al.         | Use of T530 HST on calcium carbonate-containing papers, Stever R. Boone, 1996, Tappi Journal, pp. 122-124.                                   |            |                  |          |  |  |
| 7,655,287 B2          | 2/2010 Yoshida et al.      | Tracing Tecniue in Geohydrology by Werner Kass and Horst Behrens, published by Taylor and Francis, 1998, pp. 48-55.                          |            |                  |          |  |  |
| 7,658,981 B2          | 2/2010 Ternmae             | Synthetic Detergents in the Soap Industry Lime Soap Dispersion Test, H.C. Borghetty et al., J. Am. Oil, Chem. Soc., 27:88-90, 1950.          |            |                  |          |  |  |
| 8,012,551 B2          | 9/2011 Song et al.         | Lipids in Cereal Staraches, A Review; William R. Morrison; Journal of Cereal Science 8 , 1988, pp. 1-15.                                     |            |                  |          |  |  |
| 8,123,907 B2          | 2/2012 Stoffel et al.      | High Solids Modified Calcium Carbonates A Concept for Inkjet Papers, Varney and Kukkamo, May 2010.                                           |            |                  |          |  |  |
| 2003/0227531 A1       | 12/2003 Hosoi              | Pigment Coating Techniques, Chapter 24, p. 415-417, Jukka Linnonmaa and Michael Trefz.                                                       |            |                  |          |  |  |
| 2005/0100688 A1       | 5/2005 Nakano et al.       | Smook, Handbook for Pulp and Paper Technologist, 2nd edition, chapter 18, pp. 283-296—1992.                                                  |            |                  |          |  |  |
| 2005/0124755 A1       | 6/2005 Mitchell            | *                                                                                                                                            |            |                  |          |  |  |
| 2006/0003117 A1       | 1/2006 Superka et al.      |                                                                                                                                              |            |                  |          |  |  |
| 2006/0051528 A1       | 3/2006 Ogino               |                                                                                                                                              |            |                  |          |  |  |
| 2006/0137574 A1       | 6/2006 Preston et al.      |                                                                                                                                              |            |                  |          |  |  |
| 2006/0254738 A1       | 11/2006 Anderson           |                                                                                                                                              |            |                  |          |  |  |
| 2007/0087134 A1       | 4/2007 Tyan et al.         |                                                                                                                                              |            |                  |          |  |  |
| 2007/0087138 A1       | 4/2007 Koenig et al.       |                                                                                                                                              |            |                  |          |  |  |
| 2007/0125267 A1       | 6/2007 Song et al.         |                                                                                                                                              |            |                  |          |  |  |
| 2007/0218222 A1       | 9/2007 Campbell et al.     |                                                                                                                                              |            |                  |          |  |  |
| 2008/0020152 A1       | 1/2008 Watanabe et al.     |                                                                                                                                              |            |                  |          |  |  |
| 2008/0098931 A1       | 5/2008 Skaggs et al.       |                                                                                                                                              |            |                  |          |  |  |
| 2008/0187691 A1       | 8/2008 Osgood et al.       |                                                                                                                                              |            |                  |          |  |  |
| 2009/0035478 A1       | 2/2009 Zhou et al.         |                                                                                                                                              |            |                  |          |  |  |
| 2009/0122127 A1       | 5/2009 Baker               |                                                                                                                                              |            |                  |          |  |  |
| 2009/0274855 A1       | 11/2009 Koenig et al.      |                                                                                                                                              |            |                  |          |  |  |
| 2009/0295892 A1       | 12/2009 Akiyama            |                                                                                                                                              |            |                  |          |  |  |

\* cited by examiner

**FIG. 1**

**FIG. 2**



**FIG. 3**

## 1

**COATED PRINTABLE SUBSTRATES  
RESISTANT TO ACIDIC HIGHLIGHTERS  
AND PRINTING SOLUTIONS**

**FIELD OF THE INVENTION**

The present invention broadly relates to printable substrates comprising paper substrates having a coating on one or both surfaces of the paper substrate which are resistant to damage which may be caused by acidic highlighters, as well as acidic printing solution used in offset printing processes. The present invention further broadly relates to a method for preparing such coated paper substrates.

**BACKGROUND**

In conventional calendered papermaking for providing papers used in printing, a fibrous web may be prepared from an aqueous solids mixture which may comprise wood pulp and/or synthetic fibers along with various additives. These additives may include paper pigment(s) such as calcium carbonate, clay, titanium dioxide, etc., as well as pigment binders such as modified starch, styrene butadiene rubber, polyvinyl acetate, vinyl acrylic, polyvinyl alcohol, etc. Other additives such as sizing agents, fillers, pigments, dispersants, viscosity modifiers, crosslinking agents, lubricants, etc., may also be included in preparing paper substrates.

In recent years, the use of ink-jet printing methods has been increasing at a rapid rate. Ink jet printing is a method for forming ink images on a paper substrate from deposited droplets of ink comprising dyes or pigments. This printing method enables high-speed and full-color printing to be achieved. In ink jet printing, the fine droplets of ink are sprayed or jetted from printing nozzles at a high speed so as to direct the ink droplets toward, and deposit these droplets on, the paper substrate to provide printed images on the paper substrate.

The ink used in ink jet printing may contain either dyes or pigments as print agents. In the case of inks comprising pigments, the ink may also be in the form of a pigment emulsion. The use of pigment emulsions in the ink may increase the dry time for the ink droplets deposited on the surface of the paper substrate, and may thus lead to, for example, smearing of the deposited ink droplets. Accordingly, coatings for the paper substrate have been developed to be more receptive to the ink deposited by inkjet printers.

In coating paper substrates to be more receptive to inks deposited by inkjet printers, the resulting coated papers printed with inkjet ink may be more susceptible to physical damage. For example, coatings applied to paper substrates to make them more receptive to inks deposited by inkjet printers tend to be more porous or water-swellable. That makes such porous, water-swellable coated paper substrates more vulnerable to damage resulting from contact with water. In the case of dye-based inks, such damage from post-imaging contact with water may take the form of, for example, smearing or smudging of the inkjet-printed image. Pigment-based-inks printed on such porous, water-swellable coated paper substrates may also be easily smudged or smeared by rubbing the still moist surface of the pigmented image on the coated paper substrate.

**SUMMARY**

According to a first broad aspect of the present invention, there is provided an article comprising: a paper substrate having a first surface and a second surface; and

## 2

an acid-resistant water-swellable substrate coating on at least one of the first and second surfaces which provides an ink-receptive porous surface, wherein the substrate coating comprises:

an acid-resistant water-swellable crosslinked polymer coating pigment binder matrix; and an amount of an acid-resistant coating pigment sufficient to impart a Parker Print Smoothness value of at least about 4 to the at least one of the first and second surfaces and which is dispersed in the binder matrix, wherein the acid-resistant coating pigment comprises from about 30 to 100% larger coating pigment particles having a mean particle size above about 1 micron in diameter.

According to a second broad aspect of the present invention, there is provided a method comprising the following steps:

- (a) providing a paper substrate having a first surface and a second surface; and
  - (b) treating at least one of the first and second surfaces with an acid-resistant water-swellable substrate coating to provide a printable substrate, wherein the substrate coating provides an ink-receptive porous surface, and wherein the substrate coating comprises:
- an acid-resistant water-swellable crosslinked polymer coating pigment binder matrix; and an amount of an acid-resistant coating pigment sufficient to impart a Parker Print Smoothness value of at least about 4 to the at least one of the first and second surfaces and which is dispersed in the binder matrix, wherein the acid-resistant coating pigment comprises from about 30 to 100% larger coating pigment particles having a mean particle size above about 1 micron in diameter.

**BRIEF DESCRIPTION OF THE DRAWINGS**

The invention will be described in conjunction with the accompanying drawings, in which:

FIG. 1 is a schematic diagram illustrating an embodiment of a method for treating one or both surfaces of a paper substrate with a coating composition using a metering rod size press;

FIG. 2 is a schematic diagram illustrating an embodiment of a method for treating one or both surfaces of a paper substrate with a coating composition using a horizontal flooded nip size press; and

FIG. 3 is a schematic diagram illustrating an embodiment of a method for treating one or both surfaces of a paper substrate with a coating composition using a vertical flooded nip size press.

**DETAILED DESCRIPTION**

It is advantageous to define several terms before describing the invention. It should be appreciated that the following definitions are used throughout this application.

**DEFINITIONS**

Where the definition of terms departs from the commonly used meaning of the term, applicant intends to utilize the definitions provided below, unless specifically indicated.

For the purposes of the present invention, directional terms such as "top", "bottom", "side," "front," "frontal," "forward," "rear," "rearward," "back," "trailing," "above", "below", "left", "right", "horizontal", "vertical", "upward", "downward", etc. are merely used for convenience in describing the

various embodiments of the present invention. The embodiments of the present invention illustrated in, for example, FIGS. 1-3, may be oriented in various ways.

For the purposes of the present invention, the term "printable substrate" refers to any paper substrate which may be printed on with an ink jet printing process. Printable substrates may include webs, sheets, strips, etc., may be in the form of a continuous roll, a discrete sheet, etc.

For the purposes of the present invention, the term "paper substrate" refers to a fibrous web that may be formed, created, produced, etc., from a mixture, furnish, etc., comprising paper fibers, internal paper sizing agents, etc., plus any other optional papermaking additives such as, for example, fillers, wet-strength agents, optical brightening agents (or fluorescent whitening agent), etc. The paper substrate may be in the form of a continuous roll, a discrete sheet, etc.

For the purposes of the present invention, the term "paper filler" refers commonly to mineral products (e.g., calcium carbonate, kaolin clay, etc.) which may be used in paper making to reduce materials cost per unit mass of the paper, increase opacity, increase smoothness, etc. These mineral products may be finely divided, for example, the size range of from about 0.5 to about 5 microns.

For the purposes of the present invention, the term "uncoated paper substrate" refers to a paper substrate which has 0 or substantially 0 paper surface loading of a coating present on one or both sides or surfaces of the paper substrate.

For the purposes of the present invention, the term "single-side coated paper substrate" refers to a paper substrate which has a surface loading of a coating present on one, but not both, sides or surfaces of the paper substrate.

For the purposes of the present invention, the term "double-side coated paper substrate" refers to a paper substrate which has a surface loading of a coating on both sides or surfaces of the paper substrate.

For the purposes of the present invention, the term "calendered paper" refers to a paper substrate which has been subjected to calendering to, for example, smooth out the paper for enabling printing and writing on the paper, and to increase the gloss on the paper surface. For example, calendering may involve a process of using pressure for embossing a smooth surface on the still rough paper surface. Calendering of paper may be carried out on a calender which may comprise a series of rolls at the end of a papermaking machine (on-line), or separate from the papermaking machine (off-line).

For the purposes of the present invention, the term "coating" refers to those coatings, which comprise, at minimum, an acid-resistant water-swellable crosslinked polymer coating pigment binder, and an acid-resistant coating pigment. These coatings (or compositions used to provide such coatings) may also include other optional additives, such as, for example, a metal salt drying agents, cationic dye fixing agents, optical brightening agents, fluorescent whitening agents, solvents, diluents, anti-scratch and mar resistance agents, defoamers, rheology modifiers, dispersants, surfactants, paper sizing agents, etc. The coating compositions may be formulated as an aqueous solution, an aqueous slurry, a colloidal suspension, a liquid mixture, a thixotropic mixture, etc.

For the purposes of the present invention, the term "solids basis" refers to the weight percentage of each of the respective solid materials (e.g., a metal salt drying agent; calcium carbonate pigment component; a cationic dye fixing agent; plastic pigment, surface paper sizing agent, optical brightening agent, etc.) present in the coating, coating composition, etc., in the absence of any liquids (e.g., water). Unless otherwise specified, all percentages given herein for the solid materials are on a solids basis.

For the purposes of the present invention, the term "solids content" refers to the percentage of non-volatile, non-liquid components (by weight) that are present in the coating, composition, etc.

5 For the purposes of the present invention, the term "acid-resistant" refers to substrate coatings, coating pigment binders, coating pigments, etc., which are resistant to degradation, decomposition, disintegration, dissolving, damage, etc., in the presence of acidic materials, such as acidic ink-based highlighters, acidic printing solutions, etc.

For the purposes of the present invention, the term "water-swellable" refers to a coating, binder, etc., which is able to absorb, imbibe, take up, etc., aqueous fluids, including inkjet inks, but which is not water-soluble, e.g., does not dissolve appreciable in the presence of such aqueous fluids.

For the purposes of the present invention, the term "coating pigment" refers to a material (e.g., a finely divided particulate matter) which may be used or may be intended to be used to affect the ink absorptive properties of a printable substrate.

For the purposes of the present invention, the term "acid-resistant coating pigment" refers to a coating pigment which may be acid-resistant due to the inherent properties of the materials comprising the coating pigment, how the coating pigment is prepared, synthesized, etc., by surrounding, encapsulating, enclosing, etc., a coating pigment which is not otherwise acid-resistant with an acid-resistant-coating, etc. Suitable acid-resistant coating pigments may include, for example, one or more of: clay, kaolin, silica, talc, calcined 30 clay, alumina, titanium dioxide, barium sulfate, bentonite clay, absorptive plastic pigments, calcium carbonate (such as ground calcium carbonate or precipitated calcium carbonate) provided with an acid-resistant coating or treated to be acid-resistant, etc. Some illustrative acid-resistant calcium carbonate pigments due to acid-resistant coatings and/or treatments include those prepared from a slurry of calcium carbonate particles mixed simultaneously with a solution of a zinc compound and a solution of a silica-containing substance such as water glass disclosed in U.S. Pat. No. 5,000,797 (Tokarz et 40 al.), issued Mar. 18, 1991; calcium carbonate acid-stabilized by the addition to finely divided calcium carbonate of one of a calcium-chelating agent and a conjugate base, such as sodium hexametaphosphate, followed by the addition of a weak acid, such as phosphoric acid disclosed in U.S. Pat. No. 5,043,017 (Passaretti), issued Aug. 27, 1991; those prepared from an aqueous slurry of particulate calcium carbonate with a sodium silicate solution slowly mixed in, followed by adding carbon dioxide and zinc chloride disclosed in U.S. Pat. No. 5,164,006 (Chapnerkar et al.), Nov. 17, 1992; calcium 50 carbonate in admixture with a cationic salt, together with an anionic salt, or a weak base together with a weak acid, or aluminum or magnesium hydroxide, together with a mixture of weak acids, or an aluminum salt such as aluminum sulfate, aluminum chloride, or polyaluminum chloride disclosed in U.S. Pat. No. 5,531,821 (Wu), issued Jul. 2, 1996, U.S. Pat. No. 5,593,488 (Wu), issued Jan. 14, 1997, U.S. Pat. No. 5,593,489 (Wu), issued Jan. 14, 1997, or U.S. Pat. No. 5,599,388 (Wu), issued Feb. 4, 1997; a mixture of calcium carbonate and sodium aluminate together with one or more weak acids, or calcium carbonate and sodium silicate, together with a weak acid, such as phosphoric acid, formic acid, fluoroboric acid, polyacrylic acid, or alum, or a mixture of weak acids, such as phosphoric acid and polyacrylic acid disclosed in U.S. Pat. No. 5,711,799 (Snowden et al.), issued Jan. 27, 1998, or U.S. Pat. No. 6,083,317 (Snowden et al.), issued Jul. 4, 2000; the entire contents and disclosures of the foregoing documents being herein incorporated by reference.

35 50 55 60 65 70 75 80 85 90 95 100

45 50 55 60 65 70 75 80 85 90 95 100

45 50 55 60 65 70 75 80 85 90 95 100

50 55 60 65 70 75 80 85 90 95 100

55 60 65 70 75 80 85 90 95 100

60 65 70 75 80 85 90 95 100

65 70 75 80 85 90 95 100

For the purposes of the present invention, the term "larger coating pigment particles" refers to acid-resistant coating pigment particles with a mean particle size above about 1 micron in diameter (for example, above about 4 microns in diameter). Sources of suitable larger coating pigment particles may include one or more of: ground calcium carbonate (GCC), precipitated calcium carbonate (PCC), absorptive plastic pigments, silica gels (e.g., Grace Davison Syloid W-300), kaolin, calcined clay, etc. In order to be acid-resistant, some of these larger coating pigment particles, such as GCC or PCC, may require an acid-resistant coating or may need to be treated to be acid-resistant.

For the purposes of the present invention, the term "smaller coating pigment particles" refers to acid-resistant coating pigment particles having particles about 1 micron or less in size. These smaller coating pigment particles may include, for example, ground calcium carbonate (GCC), precipitated calcium carbonate (PCC), fumed silica, such as anionic fumed silica (e.g., Degussa Aerodisp W7330N), alumina, titanium dioxide, barium sulfate, bentonite clay, etc., as well as mixtures thereof. In order to be acid-resistant, some of these smaller coating pigment particles, such as GCC or PCC, may require an acid-resistant coating or may need to be treated to be acid-resistant.

For the purposes of the present invention, the term "calcium carbonate" refers various calcium carbonates which may be used as fillers or coating pigments, such as precipitated calcium carbonate (PCC), ground calcium carbonate (GCC), modified PCC and/or GCC, etc. Calcium carbonate may be used as an acid-resistant coating pigment if provided with an acid-resistant coating or if treated to be acid-resistant.

For the purposes of the present invention, the term "precipitated calcium carbonate (PCC)" refers to a calcium carbonate which may be manufactured by a precipitation reaction and which may be used as a coating pigment. PCC may comprise almost entirely of the calcite crystal form of  $\text{CaCO}_3$ . The calcite crystal may have several different macroscopic shapes depending on the conditions of production. Precipitated calcium carbonates may be prepared by the carbonation, with carbon dioxide ( $\text{CO}_2$ ) gas, of an aqueous slurry of calcium hydroxide ("milk of lime"). The starting material for obtaining PCC may comprise limestone, but may also be calcined (i.e., heated to drive off  $\text{CO}_2$ ), thus producing burnt lime,  $\text{CaO}$ . Water may be added to "slake" the lime, with the resulting "milk of lime," a suspension of  $\text{Ca}(\text{OH})_2$ , being then exposed to bubbles of  $\text{CO}_2$  gas. Cool temperatures during addition of the  $\text{CO}_2$  tend to produce rhombohedral (blocky) PCC particles. Warmer temperatures during addition of the  $\text{CO}_2$  tend to produce scalenothedral (rosette-shaped) PCC particles. In either case, the end of the reaction occurs at an optimum pH where the milk of lime has been effectively converted to  $\text{CaCO}_3$ , and before the concentration of  $\text{CO}_2$  becomes high enough to acidify the suspension and cause some of it to redissolve. In cases where the PCC is not continuously agitated or stored for many days, it may be necessary to add more than a trace of such anionic dispersants as polyphosphates. Wet PCC may have a weak cationic colloidal charge. By contrast, dried PCC may be similar to most ground  $\text{CaCO}_3$  products in having a negative charge, depending on whether dispersants have been used. The calcium carbonate may be precipitated from an aqueous solution in three different crystal forms: the vaterite form which is thermodynamically unstable, the calcite form which is the most stable and the most abundant in nature, and the aragonite form which is metastable under normal ambient conditions of temperature and pressure, but which may convert to calcite at elevated temperatures. The aragonite form has an orthorhombic shape

that crystallizes as long, thin needles that may be either aggregated or unaggregated. The calcite form may exist in several different shapes of which the most commonly found are the rhombohedral shape having crystals that may be either aggregated or unaggregated and the scalenothedral shape having crystals that are generally unaggregated.

For the purposes of the present invention, the term "absorptive plastic pigment" (also known as "hollow sphere plastic pigments") refers to a coating pigment comprising a polymeric outer shell enclosing or encapsulating an inner void, space, cavity, etc. Sources of suitable absorptive plastic pigments are disclosed in, for example, U.S. Pat. No. 4,806,207 (Monzon et al.), issued Feb. 21, 1989; and U.S. Pat. No. 6,139,961 (Blankenship et al.), issued Oct. 31, 2000, the entire contents and disclosures of which are herein incorporated by reference.

For the purposes of the present invention, the term "acid-resistant water-swellable crosslinked polymer coating pigment binder matrix" refers to a water-swellable binder matrix for paper substrate coatings which may be used to improve the coating pigment binding strength of the coating and which is acid-resistant. Coating pigment binder matrices useful herein may comprise one or more of: water-soluble polymer binders, polymer latex binders, etc., which have been crosslinked so that the resulting binder matrix is water-swellable, but water-insoluble, and is acid-resistant.

For the purposes of the present invention, the term "water-soluble polymer binder" refers to a binding agent for coating pigments which may comprise linear, branched, or graft polymers or copolymers which contain sufficient hydrophilic segments to render the polymer water-soluble. Sources of suitable water-soluble polymer binders may include one or more of: starch binders, cellulosic binders (such as Methocel K, a cellulosic ether from Dow Chemical), polyvinyl alcohol binders (such as Elvanol 70-06, a fully hydrolyzed polyvinyl alcohol from DuPont), polyacrylic acid binders, polymethacrylic acid binders, polyvinylamine binders, polyacrylamide binders, polyether binders, sulfonated polystyrene binders, carboxylated polystyrene binders, etc.

For the purposes of the present invention, the term "starch binder" refers to a water-soluble polymer binder agent for coating pigments which comprises one or more of: starch, starch derivatives, etc. Suitable starch binders may be derived from a natural starch, e.g., natural starch obtained from a known plant source, for example, wheat, maize, potato, tapioca, etc. The starch binder may be modified (i.e., a modified starch) by one or more chemical treatments known in the paper starch binder art, for example, by oxidation to convert some of  $-\text{CH}_2\text{OH}$  groups to  $-\text{COOH}$  groups, etc. In some cases the starch binder may have a small proportion of acetyl groups. Alternatively, the starch binder may be chemically treated to render it cationic (i.e., a cationic starch) or amphoteric (i.e., an amphoteric starch), i.e., with both cationic and anionic charges. The starch binder may also be a starch converted to a starch ether, or a hydroxyalkylated starch by replacing some  $-\text{OH}$  groups with, for example,  $-\text{OCH}_2\text{CH}_2\text{OH}$  groups,  $-\text{OCH}_2\text{CH}_3$  groups (such as Ethylex 2035, an ethylated corn starch from A. E. Staley),  $-\text{OCH}_2\text{CH}_2\text{CH}_2\text{OH}$  groups, etc. A further class of chemically treated starch binders which may be used are known as the starch phosphates. Alternatively, raw starch may be hydrolyzed by means of a dilute acid, an enzyme, etc., to produce a starch binder in the form of a gum of the dextrin type.

For the purposes of the present invention, the term "polymer latex binder" refers to a binder agent for coating pigments which comprises polymer emulsions, polymer suspensions,

etc. Sources of suitable polymer latex binders may include one or more of: styrene butadiene rubber latexes (such as CP620NA from Dow Chemical), acrylic polymer latexes, polyvinyl acetate latexes, styrene acrylic copolymer latexes (such as CP6810NA from Dow Chemical), polyurethane latexes, starch/acrylic copolymer latexes, starch/styrene acrylic copolymer latexes (such as PenSize and PenCP starch/latex copolymers from Penford Products), polyvinyl alcohol (PVOH)/styrene acrylic copolymer latexes, PVOH/acrylic copolymer latexes, epoxy latexes, etc.

For the purposes of the present invention, the term "crosslinked polymer" refers to a polymer matrix which is chemically or physically crosslinked to be water-swellable, but not water-insoluble.

For the purposes of the present invention, the term "physically crosslinked" refers to a polymer matrix which is effectively crosslinked because of the structure of the polymer matrix (e.g., the presence of crystalline segments of the polymer chain, higher Tg segments of the polymer chain, hydrophobic segments of the polymer chain which are not water-soluble, etc.), and not because of chemical crosslinking. Suitable physically crosslinked polymers may include high molecular weight (entangled) starch polymers or wholly hydrolyzed polyvinyl alcohols (PVOH), which may have crystalline segments of the polymer chain which are not water-soluble at room temperature, or copolymers, such Pen-Cote, PenCP, PenSize, PenStock, etc., which are graft copolymers of starch and styrene acrylate polymers which contain styrene and/or acrylic side chains which are not water-soluble, as well as combinations or mixtures of such physically crosslinked polymers.

For the purposes of the present invention, the term "chemically crosslinked" refers to a polymer matrix which is crosslinked by the use of chemical crosslinking agents. Suitable chemically crosslinked polymers may include those which may be chemically crosslinked with, for example, glyoxals (such as Cartabond TSI from Clariant), borate salts (such as sodium tetraborate from U.S. Borax), organic titanate salts (such as Tyzor ET from DuPont), etc. (e.g., effective for those polymers having hydroxy groups such as polyvinyl alcohols, modified starches, hydroxylated acrylic polymers, or hydroxylated styrene acrylic polymers, celluloses, etc.), zirconium salts (such as EKA AZC series from Akzo Nobel) or azirdines (e.g., effective for those polymers having hydroxy and especially carboxy groups, such acrylic latexes, guar gum, carboxymethylcelluloses, styrene acrylic copolymers, polyurethanes, epoxies, etc.), etc., as well as combinations or mixtures of such chemically crosslinked polymers.

For the purpose of the present invention, the term "treating" with reference to the coatings, and compositions used to provide such coatings, may include adding, depositing, applying, spraying, coating, daubing, spreading, wiping, dabbing, dipping, etc.

For the purposes of the present invention, the term "paper substrate surface coverage" refers to amount of a coating, or composition used to provide such coatings, present on a given side or surface of the paper substrate being treated. Paper substrate surface coverage may be defined in terms of grams of composition per square meter of paper substrate (hereinafter referred to as "gsm").

For the purposes of the present invention, the term "remains predominantly on the surface(s) of the paper substrate" refers to the coating, or composition used to provide such coatings, remaining primarily on the surface of the paper substrate, and not being absorbed by or into the interior of the paper substrate.

For the purposes of the present invention, the term "coater" refers to a device, equipment, machine, etc., which may be used to treat, apply, coat, etc., the coating, or composition used to provide such coatings, to one or more sides or surfaces of a paper substrate, for example, just after the paper substrate has been dried for the first time. Coaters may include air-knife coaters, rod coaters, blade coaters, size presses, etc. See G. A. Smook, *Handbook for Pulp and Paper Technologists* (2<sup>nd</sup> Edition, 1992), pages 289-92, the entire contents and disclosure of which is herein incorporated by reference, for a general description of coaters that may be useful herein. Size presses may include a puddle size press, a metering size press, etc. See G. A. Smook, *Handbook for Pulp and Paper Technologists* (2<sup>nd</sup> Edition, 1992), pages 283-85, the entire contents and disclosure of which is herein incorporated by reference, for a general description of size presses that may be useful herein.

For the purposes of the present invention, the term "flooded nip size press" refers to a size press having a flooded nip (pond), also referred to as a "puddle size press." Flooded nip size presses may include vertical size presses, horizontal size presses, etc.

For the purposes of the present invention, the term "metering size press" refers to a size press that includes a component for spreading, metering, etc., deposited, applied, etc., the coating, or composition used to provide such coatings, on a paper substrate side or surface. Metering size presses may include a rod metering size press, a gated roll metering size press, a doctor blade metering size press, etc.

For the purposes of the present invention, the term "rod metering size press" refers to metering size press that uses a rod to spread, meter, etc., the coating, or composition used to provide such coatings, on the paper substrate surface. The rod may be stationary or movable relative to the paper substrate.

For the purposes of the present invention, the term "gated roll metering size press" refers to a metering size press that may use a gated roll, transfer roll, soft applicator roll, etc. The gated roll, transfer roll, soft applicator roll, etc., may be stationary relative to the paper substrate, may rotate relative to the paper substrate, etc.

For the purposes of the present invention, the term "doctor blade metering size press" refers to a metering press which may use a doctor blade to spread, meter, etc., the coating, or composition used to provide such coatings, on the paper substrate surface.

For the purposes of the present invention, the term "metal drying salt" refers to those metal salts which may improve the dry time of inks deposited or printed on printable substrates by ink jet printing processes. These metal drying salts comprise one or more multivalent metal drying salts, and may optionally further comprise one or more monovalent metal drying salts. The counter anions for these metal salts may include, for example, chloride, bromide, acetate, bicarbonate, sulfate, sulfite, nitrate, hydroxide, silicate, chlorohydrate, etc. The metal drying salt may be provided as an aqueous solution comprising, for example, from about 1 to about 60% (e.g., from about 10 to about 40%) of the multivalent metal drying salt.

For the purposes of the present invention, the term "multivalent metal drying salt" refers to those metal drying salts wherein the cationic moiety is a multivalent cation having a positive charge of two or more (e.g., a calcium cation, a magnesium cation, an aluminum cation, etc.) such as calcium salts, magnesium salts, aluminum salts, etc., and which are water-soluble. Suitable multivalent metal drying salts (e.g., divalent salts, trivalent salts, etc.) may include one or more of calcium chloride, calcium acetate, calcium hydroxide, cal-

cium nitrate, calcium sulfate, calcium sulfite, magnesium chloride, magnesium acetate, magnesium nitrate, magnesium sulfate, magnesium sulfite, aluminum chloride, aluminum nitrate, aluminum sulfate, aluminum chlorohydrate, sodium aluminum sulfate, vanadium chloride, etc.

For the purposes of the present invention, the term "monovalent metal drying salt" refers to those metal drying salts wherein the cationic moiety is a monovalent cation having a positive charge of one (e.g., a sodium cation, a potassium cation, a lithium cation, etc.) such as sodium salts, potassium salts, lithium salts, etc. Suitable monovalent metal drying salts may include one or more of sodium chloride, sodium acetate, sodium carbonate, sodium bicarbonate, sodium hydroxide, sodium silicates, sodium sulfate, sodium sulfite, sodium nitrate, sodium bromide, potassium chloride, potassium acetate, potassium carbonate, potassium bicarbonate, potassium hydroxide, potassium silicates, potassium sulfate, potassium sulfite, potassium nitrate, potassium bromide, lithium chloride, lithium acetate, lithium carbonate, lithium bicarbonate, lithium hydroxide, lithium silicates, lithium sulfate, lithium sulfite, lithium nitrate, lithium bromide, etc.

For the purposes of the present invention, the term "cationic dye fixing agent" refers to those cationic compounds (e.g., nitrogen-containing compounds) or mixtures of such compounds which may aid in fixing, trapping, etc., inks printed by inkjet printing processes, and which may provide other properties, including water fastness. These cationic dye fixing agents may include compounds, oligomers and polymers which contain one or more quaternary ammonium functional groups, and may include cationic water-soluble polymers that are capable of forming a complex with anionic dyes. Such functional groups may vary widely and may include substituted and unsubstituted amines, imines, amides, urethanes, quaternary ammonium groups, dicyandiamides, guanidines, biguanides, etc. Illustrative of such compounds are polyamines, polyethylenimines, polymers or copolymers of diallyldimethyl ammonium chloride (DADMAC), copolymers of vinyl pyrrolidone (VP) with quaternized diethylaminoethylmethacrylate (DEAMEMA), polyamides, polyhexamethylene biguanide (PHMB), cationic polyurethane latexes, cationic polyvinyl alcohols, polyalkylamines dicyandiamid copolymers, amine glycidyl addition polymers, poly [oxyethylene (dimethylimino) ethylene (dimethylimino) ethylene] dichlorides, etc., or combinations thereof. These cationic dye fixing agents may include low to medium molecular weight cationic polymers and oligomers having a molecular weight equal to or less than 100,000, for example, equal to or less than about 50,000, e.g., from about 10,000 to about 50,000. Illustrative of such materials are polyalkylamine dicyandiamide copolymers, poly[oxyethylene(dimethylimino)ethylene(dimethylimino)ethylene] dichlorides and polyamines having molecular weights within the desired range. Cationic dye fixing agents suitable herein may include low molecular weight cationic polymers such as polyalkylamine dicyandiamid copolymer, poly[oxyethylene (dimethylimino)ethylene(dimethylimino)ethylene] dichloride, for example, low molecular weight polyalkylamine dicyandiamid copolymers. See U.S. Pat. No. 6,764,726 (Yang et al.), issued Jul. 20, 2004, the entire disclosure and contents of which is hereby incorporated by reference.

For the purposes of the present invention, the term "opacity" refers to the ability of a paper substrate to hide things such as print images on subsequent sheets or printed on the back, e.g., to minimize, prevent, etc., show-through, etc. As used herein, opacity of the paper substrate may be measured by, for example, in terms of TAPPI opacity and show-through. TAPPI opacity may be measured by T425 om-91.

For the purposes of the present invention, the term "Parker Print Smoothness" refers to the extent to which the paper surface deviates from a planar or substantially planar surface, as affected by the depth of the paper, paper width, numbers of departure from that planar surface, etc., as measured by TAPPI test method T 555 om-99. Parker Print Smoothness values reflect the degree of "microroughness" of the substrate or coating surface. The higher the Parker Print Smoothness value, the rougher the substrate or coating surface. Conversely, the lower Parker Print Smoothness value, the smoother the substrate or coating surface.

For the purposes of the present invention, the term "print quality" refers to those factors, features, characteristics, etc., that may influence, affect, control, etc., the appearance, look, form, etc., of a printed image on the printable substrate. Print quality of a paper substrate may be measured in terms of, for example, one or more of: (1) print density; (2) print contrast; (3) dry times; (4) edge acuity; (5) color gamut; (6) color richness; (7) print gloss; (8) print mottle; and (9) color-to-color bleed. For the purposes of the present invention, print quality of the paper substrate is primarily determined herein by measuring the print density, dry time, and edge acuity of the paper substrate.

For the purposes of the present invention, the term "print density" refers to the optical density ("OD") measured by using a reflectance densitometer (X-Rite, Macbeth. Etc.) which measures the light absorbing property of an image printed on a paper sheet. For example, the higher the print density, the darker the print image may appear. Higher print densities also provide a higher contrast, a sharper image for viewing, etc. Print density is measured herein in terms of the black print density (i.e., the print density of images which are black in color). The method for measuring black print density involves printing a solid block of black color on a paper sheet, and then measuring the optical density. The printer used to print the solid block of black color on the paper sheet is an HP Deskjet 6122, manufactured by Hewlett-Packard, (or its equivalent) which uses a #45 (HP product number 51645A) black ink jet cartridge (or its equivalent). The default setting 25 of Plain Paper type and Fast Normal print quality print mode is used in printing the solid block of black color on the paper sheet. An X-Rite model 528 spectrodensitometer with a 6 mm aperture may be used to measure the optical density of the solid block of black color printed on the paper sheet to provide black print density values. The black print density measurement settings used are Visual color, status T, and absolute density mode. In general, acceptable black print density ("OD<sub>O</sub>") values for black pigment are at least about 1.45 when using a standard (plain paper, normal) print mode for the HP desktop ink jet printer and when using the most common black pigment ink (equivalent to the #45 ink jet cartridge). Some embodiments of the paper substrates of the present invention may exhibit black print density (OD<sub>O</sub>) values of at least about 1.50, for example, at least about 1.60. See 30 also commonly assigned U.S. Pat. Appln. No. 2007/0087134 (Koenig et al.), published Apr. 19, 2007, the entire disclosure and contents of which is herein incorporated by reference, which describes how to carry out this black print density test.

For the purposes of the present invention, the term "print contrast" refers to the difference in print density between printed and unprinted areas.

For the purposes of the present invention, the term "dry time" refers to the time it takes for deposited ink to dry on the surface of a printable substrate. If the deposited ink does not dry quickly enough, this deposited ink may transfer to other printable substrate sheets, which is undesirable. The percentage of ink transferred ("IT %") is recorded as a measure of the

## 11

dry time. The higher the amount of the percentage of ink transferred, the slower (worse) the dry time. Conversely, the lower the amount of the percentage of ink transferred, faster (better) the dry time. Embodiments of the paper substrates of the present invention may provide a percent ink transferred ("IT %") value equal to or less than about 65%. In some embodiments of the paper substrates of the present invention, the IT % value may be equal to or less than about 50%, for example, equal to or less than about 40% (e.g., equal to or less than about 30%).

For the purposes of the present invention, the term "ink transfer" refers to a test for determining the dry time of a printable substrate, for example, printable paper sheets. "Ink transfer" is defined herein as the amount of optical density transferred after rolling with a roller, and is expressed as a percentage of the optical density transferred to the unprinted portion of the printable substrate (e.g., paper sheet) after rolling with a roller. The method involves printing solid colored blocks on paper having a basis weight of 20 lbs/1300 ft.<sup>2</sup> (using an HP Deskjet 6122, manufactured by Hewlett-Packard, (or its equivalent) which uses a #45 (HP product number 51645A) black ink jet cartridge (or its equivalent) with the default setting of Plain Paper type and Fast Normal print quality print mode being used), waiting for a fixed amount of time, 5 seconds after printing, and then folding in half so that the printed portion contacts an unprinted portion of the paper sheet, and rolling with a 4.5 lb hand roller as for example roller item number HR-100 from Chem Instruments, Inc., Mentor, Ohio, USA. The optical density is read on the transferred ( $OD_T$ ), the non-transferred ( $OD_O$ ) portions of the block, and an un-imaged area ( $OD_B$ ) by a reflectance densitometer (X-Rite, Macbeth, Etc.). The percent transferred ("IT %") is defined as  $IT\% = [(OD_T - OD_B) / (OD_O - OD_B)] \times 100$ . See also commonly assigned U.S. Pat. Appln. No. 2007/0087134 (Koenig et al.), published Apr. 19, 2007, the entire disclosure and contents of which is herein incorporated by reference, which describes how to carry out the ink transfer test.

For the purposes of the present invention, the term "edge acuity (EA)" refers to the degree of sharpness (or raggedness) of the edge of a printed image (e.g., a printed line). Edge acuity (EA) may be measured by an instrument such as the QEA Personal Image Analysis System (Quality Engineering Associates, Burlington, Mass.), the QEA ScannerIAS, or the ImageXpert KDY camera-based system. All of these instruments collect a magnified digital image of the sample and calculate an EA value by image analysis. The EA value (also known as "edge raggedness") is defined in ISO method 13660. This method involves printing a solid line 1.27 mm or more in length, and sampling at a resolution of at least 600 dpi. The instrument calculates the location of the edge based on the darkness of each pixel near the line edges. The edge threshold may be defined as the point of 60% transition from the substrate reflectance factor (light area,  $R_{max}$ ) to the image reflectance factor (dark area,  $R_{min}$ ) using the equation  $R_{50} = R_{max} - 60\% (R_{max} - R_{min})$ . The edge raggedness may then be defined as the standard deviation of the residuals from a line fitted to the edge threshold of the line, calculated perpendicular to the fitted line. For some embodiments of paper substrates of the present invention, the EA value may be less than about 15, for example, less than about 12, such as less than about 10 (e.g., less than about 8). See also commonly assigned U.S. Pat. Appln. No. 2007/0087134 (Koenig et al.), published Apr. 19, 2007, the entire disclosure and contents of which is herein incorporated by reference, which describes how to measure edge acuity (EA) values.

## 12

For the purposes of the present invention, the term "color gamut" refers to the total collection of possible colors in any color reproduction system and may be defined by a complete subset colors. A higher color gamut value indicates a more vivid color print quality. Color gamut may be obtained by measuring the CIE L\*, a\*, b\* of a series of color blocks, including white (unprinted area), cyan, magenta, yellow, red, green, blue and black, and from these measured values, calculating a suitable color gamut. The CIE L\* represents the whiteness. The value of L\* may range from zero (representing black) to 100 (representing white or a perfectly reflecting diffuser). The value of a\* represents the degree of green/red. A positive a\* is red, while a negative a\* is green. A positive b\* is yellow, while a negative b\* is blue. The CIE L\*, a\* and b\* values may be measured by X-Rite 528 using a D65 light source and a 10-degree viewing angle.

For the purposes of the present invention, the term "color richness" refers to a more vivid or vibrant color print with high print density and high color gamut values.

For the purposes of the present invention, the term "gloss" refers to the ability of paper to reflect some portion of the incident light at the mirror angle. Gloss may be based on a measurement of the quantity of light specularly reflected from the surface of a paper specimen at a set angle, for example, at 75 degrees, such as in the case of 75 degree gloss (and as measured by TAPPI test method T 480 om-92).

For the purposes of the present invention, the term "print gloss" refers to a gloss measurement made on a printed paper substrate.

For the purposes of the present invention, the term "print mottle" refers to non-uniformity in the print image which may be due to unevenness in ink lay, non-uniform ink absorption, etc., across the printable substrate surface. Print mottle may be measured using a scanner based mottle tester such as the C3PATX03 Formation and Mottle Test with an Agfa Model DUOSCAN scanner. The printable substrate (e.g., paper sheet) sample to be tested is first printed on a test ink jet printer. The test pattern must include a block of solid black (100%) image. The color block is a square of about 20-50 mm by 20-50 mm. After 20 minutes of waiting time, or when the printed image is fully dried, the printed sample is positioned on the scanner with printed face down. The scanner is set at a resolution of 500 ppi (pixel per inch). A Verity software (Verity IA LLC, 2114 Sunrise Drive, Appleton, Wis. 54914) may be used to analyze the test data from the scanner. An appropriate dimension for testing based on the color block dimension is set. Two mottle indices may be measured: Micro Mottle Index and Macro Mottle Index. The Micro Mottle Index measures density variations within an area of 0.1 in<sup>2</sup>; while the macro mottle index measures the density variations of the averaged density values of each square of 0.1 in<sup>2</sup>. The lower the mottle index value, the better the print quality.

For the purposes of the present invention, the term "color-to-color bleed" refers to the spreading of one color ink into another color ink on paper which may reduce the resolution of the colored text and lines on a colored background. For example blue and black bars may be printed over a yellow color background. Green and black bars may be printed over magenta color background, and red and black bars may be printed over cyan color background. The smallest distance in microns between two color bars without bridging (or color intruding more than half way to the neighboring color bar) is recorded as the color-to-color bleed index. In other words, the smaller the value of color-to-color bleed, the better the print quality. Distances which may be tested include 50 microns, 100 microns, 150 microns, 300 microns, etc. In some embodiments of the present invention, the tested distance may reach

## 13

150 microns or less before bridging (bleed) occurs, which may be considered a “good” color-to-color bleed property.

For the purposes of the present invention, the term “digital printing” refers to reproducing, forming, creating, providing, etc., digital images on a printable substrate, for example, paper. Digital printing may include laser printing, ink jet printing, etc.

For the purposes of the present invention, the term “laser printing” refers to a digital printing technology, method, device, etc., that may use a laser beam to create, form produce, etc., a latent image on, for example, photoconductor drum. The light of laser beam may later create charge on the drum which may then pick up toner which carries an opposite charge. This toner may then be transferred to the paper and the resulting print image created, formed, produced, etc., fused to the printable substrate through, for example, a fuser.

For the purposes of the present invention, the term “electrophotographic recording process” refers to a process which records images on a printable substrate, such as paper, by xerography or electrophotography. In an electrophotographic process, the image is often formed on of the c by toner particles which are deposited one surface or side of the printable substrate, and are then thermally fixed and/or fused to that one surface or side of the printable substrate, for example, by heating. In electrophotographic recording, the printable substrate may have two relatively smooth or flat sides or surfaces, or may have one side or surface which is textured, uneven or nonsmooth/nonflat, while the other side or surface is relatively smooth or flat.

For the purposes of the present invention, the term “ink jet printing” refers to a digital printing technology, method, device, etc., that may form images on a printable substrate, such as a paper substrate, by spraying, jetting, etc., tiny droplets of liquid inks onto the printable substrate through the printer nozzles. The size (e.g., smaller size), precise placement, etc., of the ink droplets may be provide higher quality inkjet prints. Ink jet printing may include continuous ink jet printing, drop-on-demand ink jet printing, etc.

For the purposes of the present invention, the term “liquid” refers to a non-gaseous fluid composition, compound, material, etc., which may be readily flowable at the temperature of use (e.g., room temperature) with little or no tendency to disperse and with a relatively high compressibility.

For the purposes of the present invention, the term “viscosity,” with reference to the coating, or composition used to provide such coatings, refers to Brookfield viscosity. The Brookfield viscosity may be measured by a Brookfield viscometer at 150° F., using a #5 spindle at 100 rpm.

For the purpose of the present invention, the term “printer” refers to any device which prints an image on a printable substrate, such as a paper sheet, including laser printers, inkjet printers, electrophotographic recording devices (e.g., copiers), scanners, fax machines, etc.

For the purpose of the present invention, the term “printer pigment” may refer to either ink (as used by, for example, an inkjet printer, etc.) or toner (as used by, for example, a laser printer, electrographic recording device, etc.).

For the purpose of the present invention, the term “ink” refers to printer colorant as used by ink jet printers. The term ink may include dye-based inks and/or pigment-based inks. Dye-based inks comprise a dye which may be an organic molecule which is soluble in the ink medium. Dye-based inks may be classified by their usage, such as acid dyes, basic dyes, or direct dyes, or by their chemical structure, such as azo dyes, which are based on the based on an —N=N— azo structure; diazonium dyes, based on diazonium salts; quinone-imine dyes, which are derivates of quinine, etc. Pigment-based dyes

## 14

comprise a pigment, which is a solid colored particle suspended in the ink medium. The particle may comprise a colored mineral, a precipitated dye, a precipitated dye which is attached to a carrier particle, etc. Inks are often dispensed, deposited, sprayed, etc., on a printable medium in the form of droplets which then dry on the printable medium to form the print image(s).

For the purpose of the present invention, the term “toner” refers to printer pigment as used by laser printers. Toner is often dispensed, deposited, etc., on the printable medium in the form of particles, with the particles then being fused on the printable medium to form the image.

For the purposes of the present invention, the term “room temperature” refers to the commonly accepted meaning of room temperature, i.e., an ambient temperature of 20° to 25° C.

For the purpose of the present invention, the term “Hercules Sizing Test” or “HST” refers to a test of resistance to penetration of, for example, an acidic water solution through paper. The HST may be measured using the procedure of TAPPI Standard Method 530 pm-89. See U.S. Pat. No. 6,764,726 (Yang et al.), issued Jul. 20, 2004, the entire disclosure and contents of which is hereby incorporated by reference. The HST value is measured following the conventions described in TAPPI Standard Method number T-530 pm-89, using 1% formic acid ink and 80% reflectance endpoint. The HST value measured reflects the relative level of paper sizing present in and/or on the paper substrate. For example, lower HST values (i.e., HST values below about 50 seconds) reflect a relatively low level of paper sizing present in the paper substrate. Conversely, higher HST values (i.e., HST values above about 250 seconds) reflect a relatively high level of paper sizing present in and/or on the paper substrate. For the purposes of the present invention, an HST value in the range from about 50 to about 250 seconds is considered to be an intermediate HST value reflecting an intermediate level of paper sizing present in and/or on the paper substrate. The HST value measured also reflects both the level of both internal paper sizing, as well as the level of surface paper sizing present. But at the relatively low levels of paper sizing agents normally used in papermaking (e.g., from about 1 to about 2 lbs/ton or from about 0.04 to about 0.08 gsm for paper having a basis weight of 20 lbs/1300 ft.<sup>2</sup>), the HST value of the paper substrate primarily (if not exclusively) reflects the contribution imparted by the internal paper sizing agents (which generally increase HST values greatly even at low usage levels), rather than surface paper sizing agents (which generally increase HST values minimally at such low usage levels).

For the purpose of the present invention, the term “ink-receptive porous surface” refers to a substrate coating which is able to absorb, imbibe, take up, etc., deposited inkjet ink.

## DESCRIPTION

Embodiments of the articles of the present invention comprising the printable substrates which are resistant to damage which may be caused by being in the presence of acidic materials, such as acidic highlighters, acidic printing solution used in offset printing processes, etc. The embodiments of these printable substrates comprise a paper substrate having a first surface and a second surface. The paper substrate has an acid-resistant water-swellable substrate coating on at least one of the first and second surfaces. The substrate coating comprises: an acid-resistant water-swellable crosslinked polymer coating pigment binder matrix; and an amount of an acid-resistant coating pigment sufficient to impart a Parker Print Smoothness value of at least about 4 to the at least one

## 15

of the first and second surfaces and which is dispersed in the binder matrix. The acid-resistant coating pigment comprises from about 30 to 100% (such as from about 40 to 100%) larger coating pigment particles having a mean particle size above about 1 micron in diameter. The substrate coating provides an ink-receptive porous surface and the coating pigment is in an amount sufficient to impart a Parker Print Smoothness value of at least about 4 to the at least one of the first and second surfaces, for example, in the range of from about 4 to about 12, such as from about 4 to about 8.

Embodiments of the present invention also comprise a method for preparing the printable substrate comprising the coated paper substrate. In embodiments of this method, at least one of the first and second surfaces is the paper substrate is treated with the acid-resistant water-swellable substrate coating.

Acidic materials such as acidic highlighters, as well as acidic printing solution used in offset printing processes may cause similar damage paper substrates, such as coated ink jet paper products, by smearing or smudging the inkjet ink printed on the paper substrate. These acidic materials may also dissolve paper pigments and/or fillers (e.g., calcium carbonate filler particles) which are not acid-resistant.

To avoid damage which might be caused by, for example acidic highlighter ink (or acidic offset printing solutions), in embodiments of printable substrates of the present invention, the paper substrate surface is treated with a acid-resistant but water-swellable substrate coating which is insoluble in the presence of (and may be impervious to) such acidic fluids. This may be achieved by using a substrate coating which comprises: (1) an acid-resistant water-swellable chemically or physically crosslinked polymer (or polymers) which provides an acid-resistant water-swellable pigment binder matrix; and (2) an acid-resistant coating pigment dispersed in this binder matrix. The acid-resistant coating pigment comprises a certain amount or proportion of (i.e., from about 30 to 100%) coating pigment particles above submicron in size, i.e., a mean particle size above about 1 micron in diameter, such as above about 4 microns. The substrate coating provides an ink-receptive porous surface where the amount of acid-resistant coating pigment is sufficient to imparts a Parker Print Smoothness of at least about 4 (i.e., the coating surface is not smooth), such a from about 4 to about 12 (e.g., from about 4 to about 8), and which may be achieved by using certain weight ratios of acid-resistant coating pigment to binder matrix, for example, from about 2:1 to about 20:1, such as from about 2:1 to about 10:1.

An embodiment of a method of the present invention for treating one or both surfaces of the paper substrate with a coating composition comprising one or more acid-resistant water-swellable coating pigment binders and one or more acid-resistant coating pigments is further illustrated in FIG. 1. Referring to FIG. 1, an embodiment of a system for carrying out an embodiment of the method of the present invention is illustrated which may be in the form of, for example a rod metering size press indicated generally as 100. Size press 100 may be used to coat a paper substrate, indicated generally as 104. Substrate 104 moves in the direction indicated by arrow 106, and which has a pair of opposed sides or surfaces, indicated, respectively, as 108 and 112.

Size press 100 includes a first assembly, indicated generally as 114, for applying the coating composition to surface 108. Assembly 114 includes a first reservoir, indicated generally as 116, provided with a supply of a coating composition, indicated generally as 120. A first take up roll, indicated generally as 124 which may rotate in a counterclockwise direction, as indicated by curved arrow 128, picks up an

## 16

amount of the coating composition from supply 120. This amount of coating composition that is picked up by rotating roll 124 may then be transferred to a first applicator roll, indicated generally as 132, which rotates in the opposite and clockwise direction, as indicated by curved arrow 136. (The positioning of first take up roll 124 shown in FIG. 1 is simply illustrative and roll 124 may be positioned in various ways relative to first applicator roll 132 such that the coating composition is transferred to the surface of applicator roll 132.)

10 The amount of coating composition that is transferred to first applicator roll 132 may be controlled by metering rod 144 which spreads the transferred composition on the surface of applicator roll 132, thus providing relatively uniform and consistent thickness of a first coating, indicated as 148, when 15 applied onto the first surface 108 of substrate 104 by applicator roll 232.

As shown in FIG. 1, size press 100 may also be provided with a second assembly indicated generally as 152, for applying the coating composition to surface 112. Assembly 152 includes a second reservoir indicated generally as 156, provided with a second supply of a coating composition, indicated generally as 160. A second take up roll, indicated generally as 164 which may rotate in a clockwise direction, as indicated by curved arrow 168, picks up an amount of the coating composition from supply 160. This amount of coating composition that is picked up by rotating roll 164 may then be transferred to second take up roll, indicated generally as 172, which rotates in the opposite and counterclockwise direction, as indicated by curved arrow 176. As indicated in FIG. 1 by 20 the dashed-line box and arrow 176, second take up roll 164 may be positioned in various ways relative to second applicator roll 172 such that the coating composition is transferred to the surface of applicator roll 172. The amount of coating composition that is transferred to second applicator roll 172 25 may be controlled by a second metering rod 184 which spreads the transferred composition on the surface of applicator roll 172, thus providing relatively uniform and consistent thickness of the second coating, indicated as 188, when applied onto the second surface 112 of substrate 104 by 30 applicator roll 172.

40 Referring to FIG. 2, another embodiment of a system for carrying out an embodiment of the method of the present invention is illustrated which may be in the form of, for example, a horizontal flooded nip size press indicated generally as 200. Horizontal size press 300 may be used to coat a paper web, indicated generally as 204, with a coating composition (e.g., as described in FIG. 1 above). Web 204 moves in the direction indicated by arrow 206, and has a pair of opposed sides or surfaces, indicated, respectively, as 208 and 212.

45 Horizontal size press 200 includes a first source of coating composition, indicated generally as nozzle 216, which is sprays a stream of the coating composition, indicated by 220, generally downwardly towards the surface of a first transfer roll, indicated as 232, which rotates in a clockwise direction, as indicated by curved arrow 236. A flooded pond or puddle, indicated generally as 240, is created at the nip between first transfer roll 232 and second transfer roll 272 due to a bar or dam (not shown) positioned at below the nip. Transfer roll 232 transfers a relatively uniform and consistent thickness of 50 a first coating of the coating composition, indicated as 248, onto the first surface 208 of web 204.

55 A second source of coating composition, indicated generally as nozzle 256, which is sprays a stream of the coating composition, indicated by 260, generally downwardly towards the surface of a second transfer roll, indicated as 272, which rotates in a counterclockwise direction, as indicated by 60

## 17

curved arrow 276. Transfer roll 272 transfers a relatively uniform and consistent thickness of a second coating of the coating composition, indicated as 288, onto the second surface 212 of web 204.

Referring to FIG. 3, another embodiment of a system for carrying out an embodiment of the method of the present invention is illustrated which may be in the form of, for example, a vertical flooded nip size press indicated generally as 300. Vertical size press 300 may be used to coat a paper web, indicated generally as 304, with a coating composition (e.g., as described in FIG. 1 above). Web 304 moves in the direction indicated by arrow 306, and has a pair of opposed sides or surfaces, indicated, respectively, as 308 and 312.

Vertical size press 300 includes a first source of coating composition, indicated generally as nozzle 316, which is sprays a stream of the coating composition, indicated by 320, generally upwardly and towards the surface of a first lower transfer roll of the roll stack, indicated as 332, which rotates in a clockwise direction, as indicated by curved arrow 336. A smaller flooded pond or puddle, indicated generally as 340, (compared to the pond or puddle 340 of horizontal size press 300) is created at the nip between lower first transfer roll 332 and second upper transfer roll 372 due to a bar or dam (not shown) positioned to right of the nip. Transfer roll 332 transfers a relatively uniform and consistent thickness of a first coating of the coating composition, indicated as 348, onto the lower first surface 308 of web 304.

A second source of coating composition, indicated generally as nozzle 356, sprays a stream of the coating composition, indicated by 360, generally downwardly and towards the surface of a second upper transfer roll, indicated as 372, which rotates in a counterclockwise direction, as indicated by curved arrow 376. Transfer roll 372 transfers a relatively uniform and consistent thickness of a second coating of the coating composition, indicated as 388, onto the upper second surface 312 of web 304.

All documents, patents, journal articles and other materials cited in the present application are hereby incorporated by reference.

Although the present invention has been fully described in conjunction with several embodiments thereof with reference to the accompanying drawings, it is to be understood that various changes and modifications may be apparent to those skilled in the art. Such changes and modifications are to be understood as included within the scope of the present invention as defined by the appended claims, unless they depart therefrom.

What is claimed is:

1. An article comprising:

a paper substrate having a first surface and a second surface; and

an acid-resistant water-swellable substrate coating on at least one of the first and second surfaces which provides an ink-receptive porous surface, wherein the substrate coating comprises:

an acid-resistant water-swellable crosslinked polymer coating pigment binder matrix; and

an amount of an acid-resistant coating pigment sufficient to impart a Parker Print Smoothness value of at least about 4 to the at least one of the first and second surfaces and which is dispersed in the binder matrix, wherein the acid-resistant coating pigment comprises from about 30 to 100% larger

## 18

coating pigment particles having a mean particle size above about 4 microns in diameter; wherein the acid-resistant coating pigment comprises one or more of: clay, kaolin, talc, calcined clay, alumina, titanium dioxide, barium sulfate, bentonite clay, or absorptive plastic pigments, wherein the substrate coating has a weight ratio of the acid-resistant coating pigment to binder matrix in the range of about 2:1 to about 20:1.

2. The article of claim 1, wherein the substrate coating is on both the first and second surfaces.

3. The article of claim 1, wherein the substrate coating has a weight ratio of the acid-resistant coating pigment to binder matrix in the range of about 2:1 to about 10:1.

4. The article of claim 1, wherein the coating pigment comprises acid-resistant clay particles, acid-resistant absorptive plastic pigment particles, or a mixture thereof.

5. The article of claim 1, wherein the binder matrix comprises one or more chemically crosslinked polymers.

6. The article of claim 1, wherein the binder matrix comprises one or more physically crosslinked polymers.

7. The article of claim 1, wherein the acid-resistant coating pigment imparts a Parker Print Smoothness value of from about 4 to about 12.

8. The article of claim 7, wherein the acid-resistant coating pigment imparts a Parker Print Smoothness value of from about 4 to about 8.

9. The article of claim 1, wherein the acid-resistant coating pigment comprises from about 40 to 100% larger coating pigment particles.

10. The article of claim 1, wherein the binder matrix comprises one or more of: water-soluble polymer binders or polymer latex binders, wherein the one or more water-soluble polymer binders or polymer latex binders have been crosslinked so that the binder matrix is water-swellable.

11. The article of claim 10, wherein the water-soluble polymer binders comprise one or more of: starch binders, cellulosic binders, polyvinyl alcohol binders, polyacrylic acid binders, polymethacrylic acid binders, polyvinylamine binders, polyacrylamide binders, polyether binders, sulfonated polystyrene binders, or carboxylated polystyrene binders.

12. The article of claim 11, wherein the water-soluble polymer binders comprise a starch binder.

13. The article of claim 10, wherein the polymer latex binders comprise one or more of: styrene butadiene rubber latexes, acrylic polymer latexes, polyvinyl acetate latexes, styrene acrylic copolymer latexes, polyurethane latexes, starch/acrylic copolymer latexes, starch/styrene acrylic copolymer latexes, polyvinyl alcohol/styrene acrylic copolymer latexes, polyvinyl alcohol/acrylic copolymer latexes, or epoxy latexes.

14. The article of claim 13, wherein the polymer latex binder comprises a styrene acrylic latex binder.

15. The article of claim 10, wherein the one or more water-soluble polymer binders or polymer latex binders are chemically crosslinked with glyoxals, borate salts, organic titanate salts, zirconium salts, or azirdines.

16. The article of claim 15, wherein the one or more water-soluble polymer binders or polymer latex binders are chemically crosslinked with a glyoxal.